

No. 807,027.

PATENTED DEC. 12, 1905.

P. L. T. HÉROULT.  
STEEL MIXING PROCESS.  
APPLICATION FILED APR. 19, 1905.

Fig. 1.



Fig. 2.



WITNESSES:

Fred White  
René P. Huine

INVENTOR:

Paul Louis Toussaint Héroult,  
By his Attorney  
Arthur C. Fraser & Co.

# UNITED STATES PATENT OFFICE.

PAUL LOUIS TOUSSAINT HÉROULT, OF LA PRAZ, FRANCE.

## STEEL-MIXING PROCESS.

No. 807,027.

Specification of Letters Patent.

Patented Dec. 12, 1905.

Application filed April 19, 1905. Serial No. 256,365.

*To all whom it may concern:*

Be it known that I, PAUL LOUIS TOUSSAINT HÉROULT, a citizen of the Republic of France, residing at La Praz, Savoie, France, have invented certain new and useful Improvements in Steel-Mixing Processes, of which the following is a specification.

For numerous reasons it is desirable in the steel industry to regulate the work so as to secure uniformity of composition and to employ an apparatus having similar functions to those exercised by the mixer which is used for cast-iron. It has not been found practicable up to the present time to use such a mixer because of the changes of composition of the bath of steel inherent in the method of heating. This heating has always been oxidizing, and consequently oxidizes the slag and burns the silicon, manganese, and carbon of the bath, so that the time and skill of the operator of the apparatus become factors of such importance as to make the process impracticable.

The process of the present invention makes possible the use of a mixer for steel preferably purified and deoxidized, substantially as usual in a Bessemer converter or other steel-making apparatus, said mixer being of considerable capacity, economical, and which not only secures uniformity in the product of an entire factory or a number of apparatus, but also secures a certain desulfurization and re-carburization and conserves the oxidizable additions—such as silicon, manganese, and the like—so as to reduce the quantities of these additions employed to a minimum. By reason of the resting of the metal at a high temperature and in very fluid condition the oxids of silicon and manganese rise to the surface, leaving a clear product.

The heat from an electric current has the prime advantage over the flames or other oxidizing methods of heating previously suggested that it is non-oxidizing. Preferably there is also maintained in the mixing-receptacle a non-oxidizing atmosphere by the introduction of an oxygen-free gas—such, for example, as producer-gas. By this neutral or reducing atmosphere the slag is maintained deoxidized, so as to favor the desulfurization of the metal and assure the conservation of the oxidizable additions referred to.

The mixer is closed, excepting only openings necessary for the repair of the linings, the entrance and discharge of the melted metal

and of the slag, and for the passage for the electrodes. The aperture through which the electrodes pass is preferably made tight by a water-cooled pressure-gasket. The openings for the doors may be made tight in any suitable way. Furthermore, the atmosphere within the furnace is maintained under pressure by the gas introduced for this purpose from a producer. Consequently when there is an opening, either accidental or intentional, at one or more of the doors there is no admission of any oxidizing element; but there is an emission at such point of a jet of flame, the extent of which can be controlled.

In the operation of an electric steel-furnace—such, for example, as the Héroult oscillating furnace shown in Patent No. 707,776, of August 26, 1902—a certain part of the energy is employed in melting or in raising the temperature of the steel already melted. The remainder is employed in compensating for the losses in radiation and convection. This fact being granted, it is apparent that by increasing the linear dimensions of the furnace (in each direction) the capacity will be increased to the third power, while the losses of heat will increase only according to the second power, according to the surface exposed. The largest charge ever smelted in an electric furnace, as far as I am aware, has been about four and one-half tons. It is proposed to make this mixer large enough to carry a charge of three or four hundred tons, to be fed by five or six Bessemer or Siemens-Martin furnaces. There are certain losses occurring in transferring the metal from the Bessemer or Siemens-Martin furnace to the electric furnace; but it is practicable to compensate for these losses very cheaply and to supply a sufficient quantity of heat for the reactions proposed, such as deoxidation and desulfurization. The difficulties to be met with in carrying out such a mixing operation for steel are not to be anticipated by a knowledge of the process of mixing pig-iron. The temperature of liquefaction of the pig-iron is about  $1050^{\circ}$  centigrade, while that of steel is  $1600^{\circ}$  to  $1800^{\circ}$  centigrade. With pig-iron it is only necessary to pour in fresh iron from the blast-furnace at sufficient intervals in order to maintain the mass in the mixer in a liquid state; but with steel it is necessary to supply additional heat, and the difficulties incidental to such a process have so far proved prohibitive. For example, an apparatus similar to that pre-

viously referred to, but larger and having a capacity of one hundred tons, will require in order to maintain its temperature at that of the fusion of steel about fifteen hundred 5 horse-power. If two thousand five hundred horse-power is furnished to the apparatus, there will remain one thousand horse-power, producing six hundred and thirty-five calories per horse-power, which places at the disposal 10 of the bath of steel six hundred and thirty-five thousand calories per hour. The specific heat of steel being about 0.25, said quantity of heat is capable of reheating through 100° for an hour about twenty-five tons of steel, which 15 we suppose to have been furnished to the mixer at a temperature already sufficient or nearly sufficient for tapping.

Instead of attaching only a secondary importance, as is the case in ordinary electric 20 furnaces, to the shape of the furnace, as it bears on the losses of heat by radiation and convection, in this mixer it is preferred to approach the form presenting the least possible surface. As the thickness of the insulating 25 materials will be likewise increased, the caloric effect will be sensibly better than that indicated.

A one-hundred-ton furnace capable of reheating through 100° twenty-five tons for an 30 hour or of reheating through 50° fifty tons for an hour fed by a two-thousand-five-hundred-horse-power generator should preferably have about the following dimensions: surface of the bath, twenty-six square meters; 35 depth, one meter. The electrodes, using a single-phase current, may be about ninety-five centimeters square in cross-section by five meters high, so as to assure their lasting six or seven weeks. With a three-phase current, 40 using three electrodes, the cross-section should be proportionally reduced.

For the operation above described one hundred kilograms of coal may be gasified in the 45 producer connected to the furnace. The mixer is preferably an oscillating apparatus, so as to permit partial pouring out of the bath. I may, however, be fixed with tap-holes at successive heights, or various other constructions 50 may be designed without changing the principle involved.

By way of example, the accompanying drawings show a receptacle having three electrodes and operating with a three-phase alternating current and in which the mixing may 55 be accomplished.

Figure 1 is a vertical section along the broken line X X of Fig. 2. Fig. 2 is a horizontal section.

Referring to the receptacle or furnace illustrated, a crucible *a* is closed by a cover *b*, through which pass three electrodes *c' c<sup>2</sup> c<sup>3</sup>*. Each of these electrodes is carried by an arm, such as *d'*, (or *d<sup>2</sup>* or *d<sup>3</sup>*), of which the support *e* is in engagement with, and may be raised 60 or lowered by means of a system of pinions

and an endless worm controlled by an electric motor *f*. Each vertical support *e* is guided by rolls *g* between U-shaped members fixed upon the heel of the crucible with interposed insulating material. Each carbon or electrode is embraced by a collar of metal sheets which is compressed or slackened by means of a screw *h*, operated by a wheel *i* through a suitable intermediate system of gearing. The crucible *a* carries also a spout *j*, through which the metal may be poured out when the furnace is inclined. There are three doors *k' k<sup>2</sup> k<sup>3</sup>*, corresponding, respectively, in position with the electrodes. The slag is ordinarily poured out of the rear doors *k<sup>2</sup>* and *k<sup>3</sup>* and the metal 70 out of the front door *k'*. The electrodes are surrounded by cooled pressure-gaskets *l*. The crucible *a* is also provided with a passage *m* in communication with a gas-producer *n*, from which the gases are led into the crucible *a*, 75 which in operation is entirely closed. The metal and slag ordinarily occupy the positions indicated in Fig. 1.

The crucible *a* carries curved tracks, which rest upon a suitable pedestal *o*, and has its 80 other point of support on the articulated piston of a hydraulic cylinder *q*, which is also articulated and which serves to determine the angle at which the crucible is tipped.

The details are represented more or less diagrammatically. They will be found described and shown more in detail in my previous patent above referred to.

It will be understood that the furnace may be operated with a two-phase or single-phase 90 current or with a continuous current and may have any suitable number of electrodes different from that indicated.

Various apparatus may be used in carrying out the process, and various modifications in 100 the details of the process may be made by those skilled in the art without departure from the invention.

What I claim is—

1. In the treatment of steel, the process of 110 mixing the products from a number of converters or the like, which consists in introducing them in a molten condition into a single receptacle, and maintaining the mass molten in said receptacle by heat from an electric 115 current, removing portions only of the composite molten contents of the receptacle without entirely emptying the same, and successively replenishing the receptacle with fresh 120 additions, whereby to secure uniformity of product from said number of converters, said process being carried on in a non-oxidizing atmosphere, whereby desulfurization and conservation of the oxidizable additions are favored.

2. In the treatment of steel, the process 125 which consists in introducing the steel, purified and deoxidized substantially as usual, and in a molten condition, into a receptacle, and maintaining it molten and in a non-oxidizing 130

atmosphere, whereby desulfuration and conservation of the oxidizable additions are favored.

3. In the treatment of steel, the process which consists in introducing the steel, purified and deoxidized substantially as usual, and in a molten condition, into a closed receptacle, maintaining it molten in said receptacle, and supplying an oxygen-free gas within the receptacle, whereby desulfuration and conservation of the oxidizable additions are favored.

4. In the treatment of steel, the process which consists in introducing the steel in a

molten condition into a receptacle, and maintaining it molten in said receptacle by the heat 15 from an electric current, said process being carried on in a non-oxidizing atmosphere, whereby desulfuration and conservation of the oxidizable additions are favored.

In witness whereof I have hereunto signed 20 my name in the presence of two subscribing witnesses.

PAUL LOUIS TOUSSAINT HÉROULT.

Witnesses:

DOMINGO A. USINA,  
FRED WHITE.